

## UNITED STATES PATENT OFFICE

2,635,045

## MAKING ELASTOMER CONTAINING PAPER

Andrew Loy Moore Bixler, Milford, N. J., and Jacob I. Fisher, Easton, Pa., assignors to Riegel Paper Corporation, New York, N. Y., a corporation of New Jersey

No Drawing. Application April 21, 1948,  
Serial No. 22,498

15 Claims. (Cl. 92—21)

1

This invention relates to improvements in the manufacture of paper having elastomeric materials incorporated therein, and more particularly to the production of a strong, tough and pliable sheet of paper with a high initial tear strength, with a soft, leather-like feel and with good abrasion resistance.

The invention includes an improved method of producing such paper and the improved paper resulting therefrom.

The invention includes an improved method of incorporating elastomeric materials to the extent of about 20% to 50% in a sheet of paper by precipitating emulsions of elastomeric materials in paper pulp which, instead of having ordinary beater consistencies of around 3 to 5% fiber solids, is diluted to a consistency of around 1% of fiber solids before the addition of the emulsions and the precipitation of the elastomeric materials therefrom; and in which the protective colloid materials are associated with the fibers, rather than with the emulsion, before the emulsion is admixed with the paper pulp and the elastomeric materials precipitated therefrom.

The invention includes further improvements in the process of making such paper in which the protective colloid materials, and advantageously also part or all of the alum for precipitating the elastomeric materials from the emulsions, are incorporated in the pulp in the beater at ordinary beater consistencies prior to dilution of the pulp to a consistency of around 1% and the admixture of the emulsions of elastomeric materials therewith.

The invention includes process steps which are advantageously utilized in combination in producing the improved and superior, tough, pliable sheet of paper with a high initial tear strength.

The process of making paper having elastomeric materials incorporated therein by precipitating rubber latex or synthetic rubber latex or emulsions of elastomeric materials in paper stock is a known process. It is also well known that the ordinary emulsions of this kind, when precipitated directly with a coagulant such as alum, tend to come out in the stock as balls or agglomerates of sticky material, whereas it is desirable that the rubber be precipitated in the form of a fine flock. If the elastomer comes out and forms balls or clots of fibers it is not uniformly distributed on the fibers even though the precipitate be finely divided and evenly distributed. The purpose of incorporating elastomeric materials in paper pulp and of producing paper having elastomeric materials incorporated therein is so that

2

a strong, tough, pliable sheet of paper may be made.

One of the chief physical properties desired in this type of paper is known and referred to in the paper trade as initial tear or edge tear. The improved process of the present invention results in the production of a superior sheet of paper having high initial tear strength as well as a soft, leather-like feel and good abrasion resistance.

10 Paper pulp or stock at ordinary beater consistencies contains around 3 to 5% of fiber solids in the fiber-water suspension.

While it is possible to obtain fair results by the use of such beater consistencies at the time of precipitation of the elastomeric material from the emulsions, we have discovered that paper with superior physical properties can be made by precipitating the rubber at a stock consistency of about 1%. We have found that a consistency of about 1% appears to be an optimum condition for the precipitation. We have found that the maximum physical properties were obtained in the range of from  $\frac{3}{4}$  of 1% to 1 $\frac{1}{2}$ % consistency, with best results at 1%; and that precipitation at materially higher or lower consistencies than these gave distinctly inferior properties to the paper.

We have also found that it is important, for best results, to associate the protective colloid materials with the fibers rather than with the emulsion before it is admixed with the fibers. This is contrary to the present procedure and to the commonly accepted teaching of the art that it is the emulsion particles which should be associated with the protective colloid materials before they are admixed with the paper stock. When the present practice is used, and the protective colloid materials are incorporated in the emulsion, an apparently uniform precipitation can be obtained without objectionable clotting of the fibers; but the precipitation of the elastomeric material, though it be in the form of a fine flock, will not be firmly and completely attached to the fibers and a product of inferior physical properties is produced.

The amount of latex or elastomeric emulsion used in making the new paper can be varied to give paper containing from about 20% to about 50%. An amount of about 30% in the paper is advantageous. Above 30% only slight additional strength or toughness is attained, but improved resistance to penetration is obtained, which is advantageous for certain uses. Below 20% the strength and toughness drop off rapidly. Such an amount of latex or elastomeric emulsion cor-

responds to from about 25% to about 100% of elastomeric material based on the dry weight of the fibers of the pulp to which the latex or emulsion is added to give paper containing from about 20% to about 50% of elastomeric material.

The improved process of the present invention will be further illustrated by the following specific example:

*Example 1.*—100 lbs. of unbleached kraft pulp were beaten to 700 cc. freeness (Canadian) in an ordinary paper mill beater. This was done at ordinary paper-making consistency (3 to 5%). The stock was then emptied to a chest and diluted to 1% consistency and the following chemicals were added as colloid protectives: 1 lb. oxalic acid dissolved in 2½ gallons of water; 1 lb. sodium hydroxide dissolved in 2½ gallons of water; 2 lbs. sodium silicate syrup (special brand) dissolved in 2½ gallons of water; .75 lb. alpha protein dissolved in 25 cc.'s of ammonium hydroxide in 2½ gallons of water; 7.2 lbs. of ammonium hydroxide (28.9%). These chemicals were thoroughly mixed with the fiber water suspension and then the elastomeric emulsion was added. In this case 154 lbs. of 27.8% solids synthetic (acrylonitrile-butadiene) rubber latex were used.

After the rubber emulsion was thoroughly mixed, alum was added to coagulate the rubber. The alum was added as a 2% solution and about 13 lbs. was necessary for complete coagulation. The preferred method was to add it in steps of 2 lbs. at a time, allowing 5 minutes between additions. Thorough mixing was obtained after and during addition. As soon as the precipitation was complete, the stock was ready to run on the paper machine.

In the above example the pulp was diluted from ordinary paper making consistency to about 1% consistency before the incorporation of the protective colloids therein. We have found, however, that the protective colloid materials can advantageously be added to the stock in the beater at ordinary beater consistencies (e. g., around 3 to 5%) and that the dilution to 1% consistency can then be made and followed by the addition of the emulsion and precipitation by alum. This procedure is more advantageous for mill operation, while the paper produced is nevertheless paper of the desired improved physical properties.

As an illustration of the improved initial tear strength of the paper obtained when the latex or elastomeric emulsion was precipitated at a consistency of 1%, according to the above example, we give below the results obtained with such precipitates in comparison with the results obtained when the latex or elastomeric emulsion was precipitated at 4% consistency.

It is evident from the above data that the initial tear is very much superior when the latex or elastomeric emulsion is precipitated in the paper pulp at 1% consistency than it is at 4% consistency.

The theory and exact mechanism of the effect of consistency on the precipitation of elastomeric materials from emulsions in paper stock, as above illustrated, and the reason for the improved results obtained at the optimum consistency of around 1%, is not yet clearly understood; but the marked improvement in results has been demonstrated. Microscopic studies of the fibers indicate that at the optimum consistency of about 1% the precipitated elastomeric particles are evenly distributed and firmly attached to the fibers. Elastomeric materials precipitated materially outside of the optimum consistency range show under the microscope more spotty distribution and poor adhesion to the fibers. At the optimum consistency the water in the slurry becomes completely clear, indicating that the elastomeric material has been finely attached to the fibers; while materially outside the optimum consistency range the water of the slurry tends to remain turbid, apparently because the elastomeric precipitate is not completely attached to the fibers, in which case the retention of the elastomeric precipitate in the sheet is dependent to a considerable degree on the filtering action as the sheet is being formed. In the optimum range, where the elastomeric material is firmly held by the fibers, apparently by some physical phenomenon, the retention of the elastomeric particles is much more positive than that obtained by simple filtering action.

While we do not desire to limit ourselves by any theoretical explanation of the mechanism or mechanics of the precipitation process, we have been led to believe that when the consistencies are materially below ¾ of 1%, the emulsion solids will precipitate mostly or to a considerable extent in the water; while with consistencies of about 1% we are led to believe that the area of total fiber exposed will be such as to allow the emulsion solids to cover each fiber evenly and that when this condition exists each individual fiber adds to the final strength of the sheet. As the consistencies rise above the optimum we are led to believe that the precipitated rubber present does not get on the fibers evenly and coats only part of the fiber surface present, e. g., around 40 to 70%, with resulting lowering of the strength of the sheet formed. It may be that the optimum consistency of about 1% is such that the fibers are so spaced apart as to promote uniform and effective precipitation of the emulsion solids on or in such

| Precipitating consistency | Basis Weight 3,000 sq. ft. | Gauge in Inches | Tensile, p. s. i. | Percent Stretch | Initial Tear Factor (Tensile $\times$ Stretch) | Hand Tear Evaluation |
|---------------------------|----------------------------|-----------------|-------------------|-----------------|------------------------------------------------|----------------------|
| 1.0%                      | 162                        | 16.5/1,000      | 2,155             | 15.4            | 33,000                                         | Good.                |
| 4.0%                      | 190                        | 21/1,000        | 1,474             | 6.0             | 8,850                                          | Poor.                |

The initial tear factor (the tensile strength multiplied by the per cent stretch) has been devised as a numerical measure of the property measured when an initial tear is made by hand. It has been found that this so-called initial tear factor, within certain limits, gives a quite satisfactory valuation of the property being evaluated when a sheet of paper is torn from a trimmed edge by hand.

intimate contact with the fibers as to give a resulting stock with the fibers so oriented therein and so intimately coated with the fine precipitated elastomer particles as to give the improved properties which we have observed are obtained in such cases.

The process described in the above example requires effective and thorough agitation during precipitation and a slow or stepwise addition of

the alum. While the improved paper of high initial tear strength can be produced in this way, we have found that the process can be further improved and simplified and paper of the desired superior properties obtained by adding both the protective colloid materials and the alum for partial precipitation to the beater while the stock is at beater consistency of around 3 to 5%. The amount of alum thus added is advantageously about one-half to four-fifths of the alum required for precipitation. This alum is added to the beater after the addition of the protective colloid materials and after these have been well mixed with the stock. This alum can be added as a 10% solution all at one step. We refer to this as the pre-alum addition.

After the pre-alum is well mixed and distributed throughout the stock, the protected stock is dumped from the beater to a chest and diluted to 1% consistency and the emulsion is then added and allowed to mix for about 15 minutes. Depending on the quantity of the pre-alum used, the elastomeric material is more or less precipitated during this mixing period. An advantageous method of procedure is to add sufficient pre-alum to precipitate about 80 to 90% of the emulsion solids. The remaining 10 to 20% is then precipitated by further addition of alum added slowly as a 1% solution.

The process carried out with the addition of both the protective colloid materials and the pre-alum to the beater before dilution is illustrated by the following example:

*Example 2.*—100 lbs. of unbleached kraft pulp were beaten to 700 cc. freeness (Canadian) in an ordinary paper mill beater at 4% consistency. The following chemicals were then added: 1 lb. oxalic acid in 2½ gallons of water; 1 lb. sodium hydroxide in 2½ gallons of water; 2 lbs. sodium silicate syrup (special brand) in 2½ gallons of water; .75 lb. alpha protein dissolved in 25 cc.'s of ammonium hydroxide in 2½ gallons of water; 7.2 lbs. of ammonium hydroxide (28-29%); and 10 lbs. alum dissolved in sufficient water to make a 10% solution. After 10 minutes' mixing, the stock was dropped from the beater to a chest and diluted to 1% consistency, then 154 lbs. of 27.8% solids synthetic rubber latex were added. After 15 minutes' mixing, 3 lbs. of alum were added slowly but continuously as a 1% solution. This completely precipitated the rubber latex and the stock was run over the paper machine, giving paper with superior physical properties.

Where alum is added following the addition of the emulsion of elastomeric materials, as in the processes above described and illustrated by the foregoing examples, it is important to insure rapid and thorough agitation. While this problem is minimized by the addition of most of the alum prior to the addition of the emulsion, it is still necessary to have rapid and thorough agitation during the addition of the small final portion of alum, after the addition of the emulsion, to complete the precipitation. In the practical carrying out of the process, the agitating equipment provided in chests may not produce sufficiently rapid and thorough agitation, since the normal operation of paper mill chests does not require such agitation. The provision of supplemental equipment to produce such agitation involves added expense and more power for its operation than the usual lower speed agitating equipment.

We have found, however, that our improved process can be carried out advantageously to pro-

duce the improved paper with high initial tear by adding all of the alum required for precipitation of the latex to the stock at beater consistency (3-5%), following the addition of the protective colloid materials and before the stock is diluted to 1% consistency prior to the addition of the rubber latex. In this modification and embodiment of the process the alum can be added dry and need not be dissolved in water before the addition to the protected stock. And we have found that this modified process is in certain respects a more simplified process and one better adapted to practical mill scale operation, and is our preferred and more practical and advantageous process.

In this improved process, in which all of the alum is added for complete precipitation of the emulsion, prior to dilution and addition of the emulsion, it is important that the quantity of alum required be determined by preliminary test, particularly as the necessary quantity of alum is somewhat flexible and varies with other factors which influence it. Thus the time, the temperature, and the degree of agitation all have influence on the quantity of alum required, all other factors being constant. This necessary quantity can be readily predetermined by test, using the pH of the stock as a measure of the amount of alum required, under the combination of other conditions existing, and maintaining the pH within narrow limits in carrying out the process.

The range of pH in which most satisfactory results have been obtained in both laboratory and commercial runs has been from about 5.0 to about 6.5, although this range does not appear to be a limiting range. We have further found that when the necessary quantity of alum has been predetermined by test, and the corresponding pH determined, it is important to control the pH within approximate  $\pm 0.2$ .

The rate of precipitation, and the time required for complete precipitation, when all of the alum is added before dilution and before the addition of the rubber latex, are important for best results. A too rapid rate of precipitation tends to cause the rubber to come out in large particles which are not firmly attached to the fibers so that a sheet of inferior strength is produced. Too slow a rate of precipitation tends to slow up production and to increase cost and to form rubber particles which though small in size are not strongly attached to the fibers, with resulting poor retention of the rubber and poor strength of the paper. We have found that the most desirable range of time for complete precipitation is from fifteen minutes to forty-five minutes, although special conditions may allow for a shorter or longer time. The rate of precipitation is also effected by other factors, such as the temperature, the degree or rate of agitation, the kind of protective colloid material used, and the quantity of protective colloid material used. However, these variables, while varying in different plants and under different conditions, will ordinarily be more or less standardized so that a preliminary test, under such standardized conditions, will enable the amount of alum required, and the corresponding pH of the stock (1%), to be predetermined so that the rate of precipitation can be controlled by controlling the pH of the stock, within rather narrow limits when the amount of alum and the corresponding pH have been so predetermined. The effect on the rate of precipitation by any of the other factors can be

compensated for by proper adjustment of the pH to predetermine the necessary quantity of alum to be added to determine the proper rate of precipitation. For example, under one condition of agitation and temperature, a pH of 5.4 may correspond to the quantity of alum required to give the proper rate of precipitation; while at another condition of agitation and temperature the same or proper rate of precipitation may be achieved at a pH of 6.2.

When the quantity of alum required for com-

with the emulsion before it is added to the paper, are shown by the following data, which illustrate the improved initial tear strength obtained when all the protective colloid materials were added to the fiber slurry in comparison with the results obtained when only half of the protective colloid materials were added to the latex or elastomer emulsion before it was admixed with the fiber slurry. All the other chemicals were added to the pulp as in the examples. In both cases the stock consistency was 1%.

| Treatment                                | Basis Wt.<br>3,000 sq.<br>ft. | Gauge in<br>Inches | Tensile,<br>p. s. i. | Percent<br>Stretch | Initial Tea<br>Factor<br>(Tensile $\times$<br>Stretch) | Hand<br>Tear<br>Evaluation |
|------------------------------------------|-------------------------------|--------------------|----------------------|--------------------|--------------------------------------------------------|----------------------------|
| All protectives added to fiber<br>slurry | 162                           | 19/1,000           | 1,750                | 18.6               | 32,600                                                 | Good.                      |
| Half of protectives added to<br>latex    | 162                           | 17.5/1,000         | 1,980                | 7.4                | 14,700                                                 | Fair.                      |

plete precipitation is thus predetermined, by test, and the corresponding pH determined, the process can be thereafter continued under the same conditions and with close regulation of the pH.

This improved process, carried out with the addition of all of the alum necessary for precipitation to the beater before dilution, is illustrated by the following example:

Example 3.—300 pounds of pulp were beaten to the desired freeness in the beater at 1.95% consistency. The following chemicals were then added: 3 pounds of oxalic acid as 16½% solution in water; 3 pounds sodium hydroxide dry flake; 18 pounds sodium silicate syrup (special brand) as received; 2½ pounds alpha protein dissolved in 75 cc. ammonium hydroxide in 17 pounds of water; 20.5 pounds of ammonium hydroxide (28-29% NH<sub>3</sub>); and 64.5 pounds of alum, dry ground. Five minutes' mixing time was allowed between each addition. Ten minutes was allowed following the addition of the alum for complete solution and mixing. The stock was then diluted to 1% consistency and dropped to a chest with 648 pounds of 20% solids synthetic rubber latex. The latex was poured down the drop line as the stock was going down. This gives rapid and thorough mixing of the latex with the completely buffered stock. The precipitation was completed in 20 minutes from the time of addition of the rubber. The pH of the buffered stock at 1% consistency just before the latex was added was 5.2.

The paper produced in accord with the above example was free from objectionable particles of rubber and had the superior physical properties, especially high initial or edge tear, shown by Examples 1 and 2. The following data are representative of paper made in accord with Example 3:

|                                                |         |
|------------------------------------------------|---------|
| Basis weight (3000 sq. ft.)                    | 282     |
| Gauge in inches                                | 21/1000 |
| Tensile, p. s. i.                              |         |
| Machine direction                              | 2500    |
| Across direction                               | 2010    |
| Per cent stretch                               |         |
| Machine direction                              | 12.0    |
| Across direction                               | 19.1    |
| Initial tear factor (tensile $\times$ stretch) |         |
| Machine direction                              | 30,000  |
| Across direction                               | 38,400  |

The improved results obtained by the process, in which the protective colloid materials are added to the fiber suspension before the emulsion is added thereto, as compared with the results obtained when the protective materials are mixed

25  
30  
35  
40  
45  
50  
55  
60  
65  
70

as "Hycar" or "Xylos" rubber. Such a synthetic rubber latex gives a resulting sheet of paper with high initial tear. The type of rubber latex to be used in carrying out the process of the invention, as well as the amount, can, however, be varied and will depend on the various properties desired in the finished sheet. Synthetic rubber latex of the type indicated is also advantageous where greaseproofness or oilproofness is required such as for gaskets. Other types of dispersions with elastomeric properties can be used, such as butadiene-styrene, neoprene, polyvinyl chloride, vinyl copolymers, nylon, and natural rubber, depending on the particular properties desired in the composite paper-elastomer sheet. Improved elastomeric properties may be obtained by the addition of suitable plasticizers with the resin, if so desired.

The examples given have referred to unbleached kraft pulp. Our invention is not, however, limited to this pulp. Other pulps suitable for paper making are included. Some such pulps are the various wood pulps (sulfite, kraft, soda, semichemical, groundwood, etc.), rag pulp, rope pulp, jute pulp, etc. Bleached or unbleached pulps are included. The exact choice of pulp and whether or not it is bleached will depend on the properties desired to fulfill the final use requirements of the paper.

Variations can be made in the process from the formulas and procedures of the above examples, which are intended to be illustrative but not limiting. Thus, for example, other colloid materials than alpha protein can be used such as, for example, hemoglobin, casein, starch, sodium alginate, etc., and these may be used in conjunction with or as substitutes for the alpha protein.

This invention includes in its scope various modifications well known among paper makers and which modifications might add desired properties for various special uses. Examples of such well known modifications that might be useful are sizing for water resistance with rosin, synthetic resin or wax, application of materials to produce wet strength, coloring, filling, calendering, embossing, etc.

It will thus be seen that the present invention provides improved processes for the production of a superior, tough, pliable paper sheet with high initial tear strength. It will also be seen that the invention includes process steps and features

which can advantageously be used in combination with each other. It will further be seen that the improved process of the invention results in the production of a new and superior sheet of paper which is strong, tough and pliable and which is characterized by high initial tear strength, a soft, leather-like feel and good abrasion resistance.

We claim:

1. In the method of making a tough, pliable sheet of paper with a high initial tear strength, having about 20% to 50% of elastomeric materials incorporated therein, the step which comprises precipitating by the action of a dilute solution of alum the elastomeric material onto the fibers of a slurry of fiber and water containing an emulsion of elastomeric material and a protective colloid material, while said slurry has a fiber consistency of about 1%.

2. The process according to claim 1 in which the protective colloid material is added to the fiber water slurry prior to the addition thereto of the emulsion of the elastomeric material.

3. The method according to claim 2 in which the precipitation of the emulsion in the slurry is effected by the stepwise addition of an alum solution containing about 2% of alum solids.

4. The method according to claim 2 in which a portion of the alum necessary is incorporated in the fiber water slurry following the addition of the protective colloid materials and prior to the addition of the emulsion of elastomeric material, the remainder of the alum necessary for precipitation being added following the addition of the emulsion of the elastomeric material, this last portion of the alum being added in dilute solution of about 2% solids concentration and in a stepwise manner.

5. The method according to claim 2 in which about four-fifths of the alum necessary is incorporated in the fiber water slurry following the addition of the protective colloid materials and prior to the addition of the emulsion of elastomeric material, the remaining one-fifth of the alum necessary for precipitation being added following the addition of the emulsion of the elastomeric material, this last portion of the alum being added in dilute solution of about 2% solids concentration and in a stepwise manner.

6. The method according to claim 2 in which all of the alum necessary for precipitation is incorporated in the fiber water slurry following the addition of the protective colloid materials and prior to the addition of the emulsion of the elastomeric material.

7. The method according to claim 2 in which all of the alum necessary for precipitation is incorporated in the fiber water slurry following the addition of the protective colloid materials and prior to the addition of the emulsion of the elastomeric material, and in which a pH of from about 5.0 to 6.5 is maintained in the slurry when the emulsion of elastomeric material is added.

8. The method according to claim 2 in which all of the alum necessary for precipitation is incorporated in the fiber water slurry following the addition of the protective colloid materials and prior to the addition of the emulsion of the elastomeric material, and in which the quantity of alum incorporated in the fiber water slurry is such as to effect precipitation of the elastomeric material from the emulsion in from 15 to 45

minutes after the addition of the emulsion to the completely buffered fiber water slurry.

9. In the method of making a tough, pliable sheet of paper with a high initial tear strength having about 20% to 50% of elastomeric materials incorporated therein, the steps which comprise adding protective colloid materials to a prepared paper stock at normal beater consistency (about 3-5%), diluting the stock to about 1% consistency, adding an emulsion of the elastomeric material to the diluted stock and precipitating the emulsion in the slurry while it is at said diluted consistency by the action of a dilute solution of alum.

10. The method according to claim 9 in which at least part of the alum is added to the stock before dilution and before the addition of the emulsion of elastomeric material.

11. The method according to claim 9 in which all of the alum necessary for precipitation is incorporated in the fiber water slurry at normal beater consistency, and the slurry is subsequently diluted to about 1% consistency before addition of the elastomeric material.

12. In the method of making a tough, pliable sheet of paper with a high initial tear strength having about 20% to 50% of elastomeric materials incorporated therein, the steps which comprise preparing a paper stock of from about 3 to 5% consistency, adding protective colloid materials thereto, subsequently adding alum thereto, diluting the stock to a slurry of fiber and water having a fiber consistency of about 1%, adding the emulsion of elastomeric material to said slurry and precipitating the emulsion therein while it is at said dilute consistency by the action of a dilute solution of alum.

13. The method according to claim 12 in which alum is also added to the diluted slurry.

14. The method according to claim 12 in which from one-half to four-fifths of the alum required for precipitation is added prior to the addition of the emulsion and in which a solution of about 2% alum is gradually added after the addition of the emulsion to complete the precipitation.

15. The method according to claim 12 in which all of the alum necessary for precipitation is incorporated in the fiber water slurry at normal beater consistency, and the slurry is subsequently diluted to about 1% consistency before addition of the elastomeric material.

ANDREW LOY MOORE BIXLER.  
JACOB I. FISHER.

55 References Cited in the file of this patent  
UNITED STATES PATENTS

| Number    | Name    | Date           |
|-----------|---------|----------------|
| 1,773,201 | Rose    | Aug. 19, 1930  |
| 1,799,217 | De Cew  | Apr. 7, 1931   |
| 2,041,968 | Schur   | May 26, 1936   |
| 2,215,553 | Johnson | Sept. 24, 1940 |
| 2,330,084 | Scott   | Sept. 21, 1943 |
| 2,474,801 | Owen    | June 28, 1949  |

65 FOREIGN PATENTS

| Number  | Country       | Date          |
|---------|---------------|---------------|
| 375,845 | Great Britain | June 30, 1932 |
| 402,982 | Great Britain | Dec. 14, 1933 |

70 OTHER REFERENCES

India Rubber World, Feb. 1, 1923, page 283.